# EUROPEAN PATENT SPECIFICATION

(11) **EP 0 657 257 B1**
(45) Date of publication and mention of the grant of the patent: **10.12.1997**
(21) Application number: 94810403.9
(22) Date of filing: 07.07.1994
(51) Int. Cl.: B27N 7/00

(54) **Wood based composite**
Zusammensgesetztes Material auf der Basis von Holz
Composite à base de bois

(30) Priority: 13.12.1993 US 166575
(43) Date of publication of application: 14.06.1995
(73) Proprietor: CANADIAN FOREST PRODUCTS LTD., Vancouver, B.C. V7X 1B5 (CA)
(72) Inventor: Chow, Suezone, Richmond, B.C. V7A 1K6 (CA); Martin, David Timothy, Langley, B.C. V3A 6G4 (CA)
(74) Representative: Kiliaridis, Constantin

(56) References cited:
- DE-A- 2 439 016
- FR-A- 2 568 510
- FR-A- 2 667 264
- US-A- 4 612 224
- DATABASE WPI Derwent Publications Ltd., London, GB; AN 92-136605 & JP-A-4 077 241 (TAKEHIRO KK) 11 March 1992
- DATABASE WPI Derwent Publications Ltd., London, GB; AN 89-066698 & JP-A-1 020 399 (NICHIHA KK) 24 January 1989

## Description

This invention relates to a method of finishing a wooden surface.

FR-A-2 667 264 discloses such a method. For the purpose of obtaining a smooth surface or a panel, solid rough wooden core layer is covered with a scrim and a mixture of wooden fibres and adhesive in a heated press.

In any industry that involves the reduction in size of non-uniform materials at high speed, particularly in saw milling, the cutting action of the tool results in very rough surfaces and variable dimensions of the cut pieces. A saw mill cutting lumber to a nominal thickness of one inch will obtain actual thicknesses ranging from 0.5 to 1.25 inches. Laminating such pieces to produce larger members for structural or decorative applications requires that the pieces be planed to uniform thickness with smooth surfaces. Failure to finish in this way will prevent the application of an adhesive or the formation of a durable bond. The cost of processing the wood to obtain the requisite surface and the amount of waste generated are both high. The processing of nominal one inch lumber to meet the adhesion requirements can result in losses of wood fibre in the range 25 to 40 percent by weight of the original wood.

The present invention seeks to provide a method of avoiding the above processing and thus the consequent waste.

The invention seeks to avoid the waste involved in the above processing and is a method of finishing a wooden surface, said method being characterized in that the mixture comprises a thermosetting adhesive, and a prefabricated needled mat comprising in addition a wooden fibre, a thermosetting resin and at least one other fibre having a longer strand length than the wood fibre.

Although the present invention is useful in finishing any wooden surface, its preferred application is in the finishing of a rough wooden surface, such as would result from a saw cut.

The thermosetting resin is preferably phenol-formaldehyde. However, other useful thermosetting adhesives include phenol-resorcinol-formaldehyde resin, resorcinol-formaldehyde resin, urea-formaldehyde resin, melamine-urea-formaldehyde resin and melamine-formaldehyde resin.

The wood fibre of the mat may be either mechanically refined without delignification or chemically refined with some degree of delignification. The wood fibre may be derived from virgin or recycled, including post-consumer, wood. In carrying out the manufacture of the wood mat, the fibre is treated with the thermosetting resin and dried. The dried, resinated wood fibre is formed into a mat in an air-laid process. This mat is intimately mixed with another mat composed of at least one other fibre. That fibre may be a synthetic material such as polyester or a polyolefin, or a natural material such as hemp, flex jute or kenaf. The two mats are blended together by passing them through a toothed roller. A fine synthetic scrim is fed onto the bottom of blended mat as a carrier and the entire mat-scrim assembly is needled to produce a string fibre mat with mechanically interlocked wood and synthetic fibre.

In practising the invention the combined fibre mat is placed on top of lumber, for example nominal one inch thick pieces of spruce - pine - fir (SPF) as commonly produced in Western Canada. A layer of the thermosetting adhesive is applied between the two layers. The mat is transferred to a heated platen press which bonds the materials of the mat and bonds the mat to the lumber substrate. In general the pressing conditions are chosen such that compression of the lumber substrate is minimized while the fibre layer is compressed to a density of up to 1.2 g/cm².

### DESCRIPTION OF THE DRAWINGS

The following examples illustrate the invention. In the drawings referred to in these examples:
Figure 1 relates thickness of the composition to the position on the wooden surface;
Figure 2 illustrates the mouldability of the composition of the present invention;
Figure 3 shows density profiles achieved on an X-ray density analyzer; and
Figure 4 relates the screw withdrawal resistance of the composition of the present invention and other, comparative materials.

### DESCRIPTION OF THE PREFERRED EMBODIMENTS

### General Procedure

Rough, kiln-dried lumber with a moisture content in the range 8 - 16%, based on the weight of dry wood, and with nominal thickness and width or 25-50 mm and 75-300 mm respectively is planed to a thickness between 14 and 38 mm. A thermosetting adhesive layer, containing phenol-formaldehyde, phenol-resorcinol-formaldehyde, resorcinol-formaldehyde, urea-formaldehyde, melamine-urea-formaldehyde or melamine-formaldehyde resin but preferably comprising a) a commercially available phenol-formaldehyde resole resin, b) wood flour, c) wheat flour, d) soda ash and e) water, is applied at a rate of about 0.244-0.489 kg/m² to both faces of the lumber. On top of the adhesive is placed a pre-formed mat consisting of a) refined wood fibre (80-90%); b) phenol-formaldehyde or urea-formaldehyde thermosetting resin (4-9%); and c) polyester, thermoplastic or natural fibre (4-12%). The combined five element construction, comprising from top to bottom, fibre mat, adhesive, lumber, adhesive, fibre mat is consolidated and cured in a flat platen hot press. The platens are heated to a temperature in the range 150-250°C. The platens are closed at a rate of 20-40 mm/sec to a separation of 140-240% of the final thickness of the product and at a rate of 1-10 mm/sec until the maximum pressure is obtained. The final position is chosen so as to allow fibre layer thicknesses of 2-6 mm. The maximum pressure exerted on the board is in the range 20-30 kg/cm². The total press time, daylight to daylight, ranges from 2-3.5 minutes and includes from 0-4 breathing cycles of 5 to 15 seconds, which prevents steam pressure from causing inter- or intra-laminar rupturing of the elements and are achieved by opening and re-closing the press. At the end of the pressing cycle, the platens are separated to allow the finished boards to be removed from the press. The boards are subsequently stacked together so as to cool slowly to room temperature and allow complete curing of the adhesive.

The following examples illustrate the invention more specifically.

### Example 1

### New Composite Products

Four 16 inch lengths of clear kiln-dried SPF lumber with a moisture content in the range 8-16% and with nominal thickness and width of 1 inch and 4 inches respectively were planed to a thickness of 14 mm. A layer of thermosetting adhesive as described in Table 1 was applied at a rate of 0.244 kg/m² to both faces of each piece of lumber at room temperature. On top of each glued face was placed a similarly sized section of preformed fibre mat from Canadian Forest Products Ltd.'s Panel and Fibre Division. The basis weight of the fibre mat was 2.4 kg/m² and the thickness was 25.4 mm. The four sets of combined elements were placed in a hot press with 16 x 18" platens heated to 205°C. The platens were closed at a rate of 27 mm/sec to a separation of 45 mm and then at a rate of 3 mm/sec to a pressure of 24 kg/cm². The minimum separation of the platens was governed by a pair of aluminum bars of 19.0 mm thickness on the sides of the bottom platen. Once the pressure reached the maximum value, a timer was started. The pressure was maintained to an elapsed time of 60 seconds before the platen separation was increased to allow venting of the steam pressure. This opening and the subsequent closing was completed at an elapsed time of 65 seconds. The pressure was maintained again at 24 kg/cm² until an elapsed time of 90 seconds when the pressure was again removed and reapplied. This was completed at an elapsed time of 95 seconds. The maximum pressure was then maintained until an elapsed time of 120 seconds when the platen separation was increased and returned to 19.0 mm by an elapsed time of 125 seconds. At an elapsed time of 150 seconds, the platens were separated to allow removal of the pressed boards. The boards were stacked on top on one another to retain heat and complete the cure of the adhesive.

The difference between the lumber thickness and the thickness of the product is accounted for by the pressed fibre, neglecting any compression of the lumber substrate. In this example the target thickness of the fibre layer in the finished product was 2.5 mm. This corresponds to a density of that layer of ca. 1.0 g/cm³.

This example demonstrates the feasibility of using fibre mats for overlaying solid wood substrates.

**Table 1**

| Phenol-Formaldehyde Thermosetting Adhesive | |
|---|---|
| Liquid Resole Resin | 43.70 |
| Water | 14.31 |
| Wood Flour | 7.31 |
| Wheat Flour | 5.91 |
| Soda Ash | 1.97 |
| Mix for 20 minutes | |
| Liquid Resole Resin | 19.81 |
| Water | 6.99 |
| Mix for 5 minutes | |
| Total | 100.00 |

### Example 2

### SPF Lumber with Various Thickness Profiles

Example 1 described the preparation of the new composite using smooth, planed lumber as the substrate. One of the main advantages of this invention is the ability of the fibre mat to mould to the shape of the lumber substrate and effectively mask any thickness variations or extreme roughness. It is a desirable feature of the invention that large variations in the thickness of the substrate can be tolerated without impairing the bonding at the solid wood/fibre interface.

To illustrate this point, some samples of the composite were prepared from lumber that had been analyzed with a custom built laser-based thickness scanner. The system consisted of a conveyor, laser heads and sensors mounted above and below the conveyor, data acquisition card, encoder and personal computer. The lumber thicknesses were determined by subtracting the sum of the distance from the bottom laser head to the bottom of the board and the distance from the top laser head to the top of the board from the total distance between the laser heads. This technique allowed non-contact measurement unaffected by any vertical board movement. In this manner, the data depicted in Figure 1 were collected from 4 pieces of lumber. Board 1 was a sample of rough, unplaned 1x4 SPF with an average thickness of approximately 28.5 mm from a Canadian Forest Products sawmill in northern British Columbia. Board 2,3,4, were from the same source but had been planed in the laboratory to average thickness of ca. 27.4, 25.1, 22.1 mm respectively.

These boards were overlaid with wood/polyester fibre mat using the conditions described in Example 1. Inter-laminar adhesion of the pressed composite were evaluated using a modification of ASTM D 2338-82, Standard Test Method for Strength Properties of Adhesives in Two-Ply Wood Construction in Shear by Tension Testing in which the samples were sliced so that the lumber remaining was the same thickness as the pressed fibre layer. In this way, each glueline could be evaluated as two-ply construction. The results of the shear testing are shown in Table 2 and reveal that the strength of the inter-laminar bond does not depend on the average thickness or the thickness profile. At the end of the test, the broken samples were inspected and the reason for the breakage was determined by visual inspection and ascribed to solid wood failure, fibre mat failure, glueline failure or a combination thereof. The amount of glueline failure during the test is very small in all cases.

This example demonstrates that lumber thickness and surface roughness are not key determinants of the integrity of the present invention and that smooth lumber surfaces, usually of vital importance to the bond quality of laminated wood composites, is not required in the invention.

**Table 2**

| Specimen Number | Condition | Lumber Thickness (mm) | Fibre Thickness (mm) | Composite Thickness (mm) | Shear Avg (psi) | Standard Deviation (psi) | Glueline ¹ Failure (%) |
|---|---|---|---|---|---|---|---|
| 0 | Rough | 28.45 | 5.08 | 33.53 | 246 | 29 | 0 |
| 1 | Planed | 27.35 | 5.08 | 32.43 | 240 | 36 | 1 |
| 5 | Planed | 25.08 | 5.08 | 30.16 | 228 | 33 | 5 |
| 6 | Planed | 22.10 | 5.08 | 27.18 | 251 | 22 | 9 |

| | | | | | | | |
|---|---|---|---|---|---|---|---|
| 1. Determined by visual inspection of the tested samples. Breakage was described as occurring in the fibre layer, in the wood layer or at the glueline. | | | | | | | |

### Example 3

### Density Profile Measurements

Lumber thickness variations such as those described in Example 2 are compensated for in this invention by the mouldability of the fibre mat which allows the fibre to fill depressions and voids in the lumber surface. As a result, the density of the fibre layer is lower in density in such areas.

To demonstrate this property, some composite samples, as shown in Figure 1, were prepared from lumber 10, machined to create some exaggerated thickness changes as shown at 12, and mat 14. In the samples prepared distance D was 1.5, 3.0, 4.5 or 6mm. Finished height H was 36mm. These samples were analyzed on a Recon Model 8900/DA X-Ray Density Analyzer and the resultant density profiles are shown in Figure 2. The sample with the shallowest depression (40X) clearly shows 3 distinct density ranges. In the middle, the density is constant at approximately 0.40 g/cm³ which corresponds to the density of the lumber substrate. On each face, there is a high density region resulting from the pressed fibre mat. In each of these fibre areas there is also some density variation as the density in the middle of the region is lower than the density either at the lumber interface or the surface that would have been next to the platen during pressing. The density profile of the fibre layers changes as the depth of the depressions becomes greater (Samples 50x, 60x and 70x). In these cases, the average density of the fibre regions lowers considerably on the side containing the depression. In fact in the extreme cases, the density of the fibre layer is lower than that of the lumber. However, there are also some noticeable changes in the fibre layer on the side opposite to the depression. In this case there is also a lowering in average density and the density profile across the fibre layer becomes more pronounced. Therefore, the conclusion is that both fibre layers assist in masking a defect on one of the faces.

Another advantage of this invention is that the average density is considerably lower than other wood-based composites such as particleboard or medium density fibreboard. This is advantageous from the point in view of the user (e.g. better machinability and lower shipping costs) and the producer (e.g. increased fibre utilization). However, the composite does have a high surface density of up to 1.0 g/cm³. In fact, it is possible, by changing the fibre layer thickness, to alter the surface density to produce a desired surface property. This is important since the surface qualities (e.g. bending strength - see Table 4 - abrasion resistance and paintability) depend on surface density.

The above example demonstrates why the strength to weight ratios of the present invention are superior to other wood based composites such as particleboard or medium density fibreboard. In simple terms, the product can be described as being "strong and light".

### Example 4

### Other Processing Parameters

The procedure of Example 1 was repeated several times with the following changes being made: 1) the total time in the hot press was varied from 1.75 to 2.75 minutes and 2) the open assembly time (i.e. the amount of time from the application of the adhesive to the lumber substrate and the mating of the fibre mat to that layer) was varied from 0 to 20 minutes. The pressed samples were tested for inter-laminar adhesion using ASTM D 2339-82, Standard Test Method for Strength Properties of Adhesives in Two-Ply Wood Construction in Shear by Tension Testing. The samples were tested for shear values and position of failure (either glueline, wood or fibre). The results, as shown in Table 3, show that 2.50 minutes press time appears to be the optimum condition for this combination of materials as the shear values are near the maximum and the glueline failure is near the minimum for all assembly times. However, the product will tolerate other processing parameters required by available species, materials, equipment or ambient conditions.

**Table 3**

| Inter-Laminar Adhesion of Fibre Mat Overlaid SPF | | | | |
|---|---|---|---|---|
| Sample | Open Time (min) | Press Time (min) | Stress Average (psi) | Glueline Failure (%) |
| A | 0 | 1.75 | 136 | 94 |
| | 5 | | 198 | 48 |
| | 10 | | 171 | 50 |
| | 15 | | 197 | 50 |
| | 20 | | 189 | 25 |
| B | 0 | 2.00 | 148 | 75 |
| | 5 | | 92 | 68 |
| | 10 | | 238 | 06 |
| | 15 | | 202 | 06 |
| | 20 | | 223 | 12 |
| C | 0 | 2.25 | 164 | 50 |
| | 5 | | 89 | 63 |
| | 10 | | 217 | 00 |
| | 15 | | 237 | 00 |
| | 20 | | 220 | 00 |
| D | 0 | 2.50 | 237 | 01 |
| | 5 | | 233 | 00 |
| | 10 | | 229 | 00 |
| | 15 | | 214 | 00 |
| | 20 | | 225 | 00 |
| E | 0 | 2.75 | 239 | 00 |
| | 5 | | 207 | 00 |
| | 10 | | 245 | 00 |
| | 15 | | 236 | 00 |
| | 20 | | 216 | 01 |

### Example 5

### Incorporation of Other Natural Fibres

The above examples describe the use of fibre mats composed of a mixture of natural wood and synthetic (polyester) fibres. However, it is possible to replace the synthetic fibre with other, natural materials such as flax. In a typical experiment, resinated hemlock fibre used in production of Woodmat at Canadian Forest Products Ltd.'s Panel and Fibre Division (90%) was combined with flax fibre (10%) cut to approximately 7.5 cm in length. The flax (237.84g, 11.9% moisture) and hemlock (2156.88g, 11.9% moisture) fibre were blended in a static Littleford mixer for 10 minutes. A portion (89.23g) of the blended fibre was formed into a mat on each side of a 16" section of SPF 1x4 that had previously been coated with the adhesive described in Example. 1. The resulting billet was pressed under the same conditions as those used for the polyester containing mats. The flexural (Modulus of Rupture = 9400 psi, Modulus of Elasticity = 1066000 psi) and lap shear properties (Stress = 200 psi) were in the same range as those obtained for polyester-containing samples.

The above example demonstrates that fibres, other than polyester, that possess a length to width ratio and good tensile strength can be used to prepare the composite.

### Example 6

### Strength Properties

Test methods were taken from ASTM D1037-87, Standard Methods of Evaluating the Properties of Wood-Base Fibre and Particle Panel Materials and ASTM D143-83, Standard Methods of Testing Small Clear Specimens of Timber. The Screw Withdrawal test was adapted for use with 19 mm material by prorating the lead hole and screw insertion depths to 12.75 mm. The material prepared as described in Example 1 was compared with other wood composite materials such as a) hardwood plywood b0 a composite comprised of a softwood veneer crossband laminate over a particleboard core c) particleboard, and d) medium density fibreboard. These samples were obtained from commercial supplies and are believed to be representative of products generally used in the marketplace. The results are shown in Table 4 and demonstrate the superiority of the present invention over currently available wood base composites as it is up to 2-3 times stronger than some other composites.

**Table 4**

| Physical Properties of Wood Based Composites | | | | |
|---|---|---|---|---|
| Type | Density (g/cm^3) | Modulus of Rupture (psi) | Modulus of Elasticity (psi) | Edge Screw Retention (lb) |
| Hardwood Plywood | 0.523 | 6430 | 580800 | 140 |
| Particleboard/Veneer Composite | 0.585 | 4160 | 306300 | 90 |
| Paticleboard | 0.720 | 1700 | 327800 | 80 |
| Medium Density Fibreboard | 0.746 | 4990 | 455600 | 130 |
| Oriented Standboard | 0.649 | 2420 | 325600 | 150 |
| Present Invention | 0.538 | 7690 | 685300 | 200 |

### Example 7

### Retention of Screw Withdrawal Resistance

As an extension of the Screw Withdrawal results described in Example 2, the ability of the materials to retain withdrawal resistance after multiple failures was investigated. The test consisted of applying load to the screw until failure, reinserting the screw to the initial depth and retesting the sample. This was repeated up to 5 reinsertions. The results are graphically displayed in Figure 4 and show that even after 5 reinsertions this invention offers withdrawal resistance superior to the initial resistance of any of the other composites. Since fastener retention is an important property of materials used in the manufacture of furniture, casegoods and cabinets, this invention should find applications in those areas.

Although the forgoing invention has been described in some detail by way of illustration and example for purposes of clarity of understanding, it will be readily apparent to those of ordinary skill in the art in light of the teachings of this invention that certain changes and modifications may be made thereto without departing from the spirit or scope of the appended claims.

## Claims

1. A method of finishing a wooden surface, said method comprising applying to the surface a mixture comprising an adhesive wooden fibre and applying heat and pressure to bond the components to each other and the wooden surface, characterized in that the mixture comprises a thermosetting adhesive, and a prefabricated needled mat comprising in addition a wooden fibre, a thermosetting resin and at least one other fibre having a longer strand length than the wood fibre.

2. A method as claimed in claim 1 in which the thermosetting adhesive is a phenol-formaldehyde resin.

3. A method as claimed in claim 1 in which the thermosetting adhesive is selected from the group consisting of phenol-resorcinol-formaldehyde resin;
resorcinol-formaldehyde resin;
urea-formaldehyde resin;
melamine-urea-formaldehyde resin and melamine-formaldehyde resin.

4. A method as claimed in claim 1 in which the thermosetting adhesive comprises a phenol-formaldehyde resin, wood flour, wheat flour, soda ash and water.

5. A method as claimed in one of claims 1 to 4 in which the thermosetting adhesive is applied to the wooden surface at a rate of about 0.244 to 0.489 kg/m².

6. A method as claimed in one of claims 1 to 5 in which the wood fibre of the mat is refined wood fibre.

7. A method as claimed in one of claims 1 to 6 in which the thermosetting resin of the mat is phenol-formaldehyde or urea-formaldehyde resin.

8. A method as claimed in one of claims 1 to 7 in which said at least one other fibre has a length in the range 50 - 100 mms.

9. A method as claimed in claim 8 in which said at least one other fibre is a synthetic fibre selected from polyester and polyolefin fibres.

10. A method as claimed in claim 8 in which said at least one other fibre is hemp or flax.

11. A method as claimed in claim 1 in which the wood fibre and said at least one other fibre are intimately mixed.

12. A method as claimed in one of claims 1 to 11 in which the mat comprises about 80-90% of the wood fibre; about 4-9% of the thermosetting resin and about 4-12% of the at least one other fibre.

13. A method as claimed in one of claims 1 to 12 in which the heat and pressure are applied by the use of heated platens.

14. A method as claimed in claim 13 in which the platens are heated to a temperature in the range 150° to 250°C.

15. A method as claimed in one of claims 1 to 14 in which the maximum pressure exerted is in the range 20 - 30 kg/cm².

16. A method as claimed in one of claims 1 to 15 in which the heat and pressure are applied for a time in the range 2 - 3.5 minutes including breathing cycles to release steam pressure.

17. A method as claimed in one of claims 1 to 16 used to treat at least two surfaces of a piece of lumber.

## Patentansprüche

1. Verfahren zur Endbearbeitung einer Holzoberfläche, wonach auf die Oberfläche eine Mischung aus Klebemittel und Holzfaser aufgebracht sowie Hitze und Druck angewendet wird, um die Komponenten miteinander und mit der Holzoberfläche zu verbinden, dadurch gekennzeichnet, dass die Mischung ein in der Wärme aushärtbares Klebemittel und eine vorgefertigte genadelte Matte aufweist, die zusätzlich eine Holzfaser, ein wärmeaushärtbares Harz und wenigstens eine weitere Faser aufweist, die eine grössere Litzenlänge als die Holzfaser hat.

2. Verfahren nach Anspruch 1, wobei das wärmeaushärtbare Klebemittel ein Phenolformaldehydharz ist.

3. Verfahren nach Anspruch 1, wobei das wärmeaushärtbare Klebemittel aus der Gruppe ausgewählt wird, welche Phenol-Resorcin-Formaldehyd-Harz;
Resorcin-Formaldehyd-Harz;
Harnstoff-Formaldehyd-Harz;
Melamin-Harnstoff-Formaldehyd-Harz und Melamin-Formaldehyd-Harz umfasst.

4. Verfahren nach Anspruch 1, wobei das wärmeaushärtbare Klebemittel ein Phenolformaldehydharz, Holzmehl, Weizenmehl, kalzinierte Soda und Wasser enthält.

5. Verfahren nach einem der Ansprüche 1 bis 4, wobei das wärmeaushärtbare Klebemittel auf die Holzoberfläche mit ungefähr 0,244 bis 0,489 kg/m² aufgebracht wird.

6. Verfahren nach einem der Ansprüche 1 bis 5, wobei die Holzfaser der Matte veredelte Holzfaser ist.

7. Verfahren nach einem der Ansprüche 1 bis 6, wobei das aushärtbare Harz der Matte Phenolformaldehyd- oder Harnstoff-Formaldehyd-Harz ist.

8. Verfahren nach einem der Ansprüche 1 bis 7, wobei die wenigstens eine Faser eine Länge im Bereich 50 bis 100 mm hat.

9. Verfahren nach Anspruch 8, wobei die wenigstens eine Faser eine synthetische Faser ist, die aus Polyester- und Polyolefinfasern ausgewählt ist.

10. Verfahren nach Anspruch 8, wobei die wenigstens eine Faser aus Hanf oder Flachs besteht.

11. Verfahren nach Anspruch 1, wobei die Holzfaser und die wenigstens eine Faser intensiv gemischt sind.

12. Verfahren nach einem der Ansprüche 1 bis 11, wobei die Matte ungefähr 80 bis 90% der Holzfaser, ungefähr 4 bis 9% des wärmeaushärtbaren Harzes und ungefähr 4 bis 12% der wenigstens einen Faser enthält.

13. Verfahren nach einem der Ansprüche 1 bis 12, wobei die Wärme und der Druck unter Verwendung erhitzter Andruckplatten angewendet werden.

14. Verfahren nach Anspruch 13, wobei die Andruckplatten auf einen Temperaturenbereich 150° bis 250°C erhitzt werden.

15. Verfahren nach einem der Ansprüche 1 bis 14, wobei der ausgeübte maximale Druck im Bereich 20 bis 30 kg/cm² liegt.

16. Verfahren nach einem der Ansprüche 1 bis 15, wobei die Hitze und der Druck während einer Zeitspanne von 2 bis 3,5 Minuten ausgeübt werden, einschliesslich von Entlüftungszyklen zur Freigabe des Dampfdrucks.

17. Verfahren nach einem der Ansprüche 1 bis 16, angewendet zum Behandeln wenigstens zweier Oberflächen eines Nutzholzstückes.

## Revendications

1. Procédé de finition d'une surface en bois, ledit procédé comprenant l'application sur la surface d'un mélange comprenant une fibre de bois adhésive et l'application de chaleur et de pression pour coller les composants l'un à l'autre et à la surface en bois, caractérisé en ce que le mélange comprend un adhésif thermo-formable, et un mat préfabriqué comprenant en plus une fibre en bois, une résine thermo-formable et au moins une autre fibre ayant une longueur de fil plus longue que celle de la fibre de bois.

2. Procédé selon la revendication 1 selon lequel l'adhésif thermo-formable est une résine formaldéhyde phénolique.

3. Procédé selon la revendication 1 selon lequel l'adhésif thermo-formable est choisi dans un groupe comprenant de la résine résorcine-formaldéhyde phénolique; de la résine résorcine-formaldéhyde; de la résine urée-formaldéhyde; de la résine mélamine-formaldéhyde et de la résine mélamine-formaldéhyde.

4. Procédé selon la revendication 1 selon lequel l'adhésif thermo-formable comprend une résine formaldéhyde-phénolique, de la farine de bois, de la farine de froment, de la soude à l'ammoniaque de commerce et de l'eau.

5. Procédé selon l'une des revendications 1 à 4 selon lequel l'adhésif thermo-formable est appliqué à la surface en bois à une quantité d'environ 0.244 à 0.489 kg/m².

6. Procédé selon l'une des revendications 1 à 5 selon lequel la fibre de bois du mat est une fibre de bois épurée.

7. Procédé selon l'une des revendications 1 à 6 selon lequel la résine thermo-formable du mat est une résine formaldéhyde-phénolique ou une résine urée-formaldéhyde.

8. Procédé selon l'une des revendications 1 à 7 selon lequel au moins une autre fibre a une longueur comprise dans la fourchette de 50 à 100 mm.

9. Procédé selon la revendication 8 selon lequel au moins une autre fibre est une fibre synthétique choisie parmi les fibres polyester et polyoléfine.

10. Procédé selon la revendication 8 selon lequel au moins une autre fibre est du chanvre ou du lin.

11. Procédé selon la revendication 1 selon lequel la fibre de bois et au moins une autre fibre sont intimement mélangées.

12. Procédé selon l'une des revendications 1 à 11 selon lequel le mat comprend 80 à 90% de fibre de bois, environ 4 à 9% de résine thermo-formable et environ 4 à 12% d'au moins une autre fibre.

13. Procédé selon l'une des revendications 1 à 12 selon lequel la chaleur et la pression sont appliquées par l'utilisation de plateaux chauffés.

14. Procédé selon la revendication 13 selon lequel les plateaux sont chauffés à une température de l'ordre de 150 à 250° C.

15. Procédé selon l'une des revendications 1 à 14 selon lequel le maximum de la pression exercée est de l'ordre de 20 à 30 kg/cm².

16. Procédé selon l'une des revendications 1 à 15 selon lequel la chaleur et la pression sont appliquées pour une durée de 2 à 3,5 minutes comprenant des cycles de repos pour détendre la pression de la vapeur.

17. Procédé selon l'une des revendications 1 à 16 utilisé pour traiter au moins deux surfaces d'une pièce de bois.
